

## 1

3,364,143

## METHOD FOR IMPROVING THE WORKING PROPERTIES OF METALS

Keith Liddell Johnson, Matteson, Ill., assignor to Swift & Company, Chicago, Ill., a corporation of Illinois  
No Drawing. Continuation-in-part of application Ser. No. 177,968, Mar. 7, 1962. This application Nov. 29, 1965, Ser. No. 510,360

7 Claims. (Cl. 252—49.5)

The present application is a continuation-in-part of application Ser. No. 177,968, filed on Mar. 7, 1962, now U.S. Patent No. 3,242,200.

This invention relates to an improved method for improving the working properties of metals in operations such as rolling, drawing, extruding and stamping. More particularly, the present invention pertains to an improved method for lubricating ferrous and nonferrous metals.

Ferrous and nonferrous metals are treated at the present time with various compositions in order to reduce burring, overheating, staining and excessive wear of the metals during milling and machining operations. Commonly employed compositions in this type of lubrication include soap and fat dispersions in the lubrication of copper tubing and wire during drawing operations, nonaqueous mineral oil solutions of esters such as butyl stearate in the treatment of aluminum and its alloys, and emulsions based on petroleum sulfonates and various oils known to the art as "soluble oils" in the cutting, drilling and sawing of ferrous metals.

The above systems, as well as other lubrication systems used at present, have certain undesirable features. For example, the use of soap and fat dispersions necessitates the installation of specially baffled tanks necessary to precipitate the copper soaps formed, thereby resulting in increased production costs. Employment of nonaqueous mineral oil-butyl stearate solutions in the preparation and handling of aluminum and its alloys requires the subsequent use of a nonaqueous solvent-type cleaner which is both costly and presents occupational and fire hazards. In the working of ferrous metals, different formulations are required for various operations resulting in high cost and operating difficulties caused by water loss from emulsions by evaporation, contamination resulting in subsequent inversion of the emulsion, contamination of other systems producing difficulties elsewhere on the production line, etc.

Therefore, it can be readily seen that a method for lubricating ferrous and nonferrous metals during milling and machining operations without incurring operational and economic difficulties heretofore experienced would be highly desirable in the art.

It is therefore an object of the present invention to provide an improved method for lubricating ferrous and nonferrous metals.

It is a further object of the present invention to provide an improved method for lubricating ferrous and nonferrous metals which will not contain inherent operational and economic disadvantages heretofore experienced in the art.

Additional objects of the present invention, if not specifically set forth herein, will be readily apparent to one skilled in the art from the following detailed description of the present invention.

In general, the objects of the present invention are accomplished by lubrication of the ferrous or nonferrous metal with an aqueous dispersion of a material prepared by reacting a monohydric, non-ionic polyoxyalkylene composition with an epoxidized ester.

Generally, the compositions employed in the present invention comprise derivatives of oxirane substituted

## 2

aliphatic acids and esters wherein the oxirane group is broken and oxyalkylene containing compositions and radicals of lower polyhydric alcohol ethers are substituted on one carbon which before the reaction had formed the oxirane group and the adjacent carbon which had formed the other carbon of the oxirane group is substituted with a hydroxyl group or an oxyalkylene group.

More specifically, the compositions used in the present invention include the products resulting from the catalyzed reaction between oxirane esters of a hydrophobic character and having a molecular weight, preferably above about 200, with oxyalkylene substituted alcohols having one available hydroxyl group. Catalysts most useful in insuring the desired reaction between the hydroxyl group of the alcohol and the oxirane containing esters are the strong Lewis acids, tertiary amines and alkali metal alcoholates.

Oxirane-substituted compounds which can be employed in producing the non-polymeric surface-active materials of the invention, as has been noted previously, comprise the hydrophobic higher molecular weight organic acids and esters having one or more oxirane groups. The epoxidized triglycerides represent a very convenient source of the oxirane-substituted materials. Epoxidized animal, vegetable and marine triglycerides are well known in the art, and examples of these materials include epoxidized soybean oil, epoxidized linseed oil, epoxidized safflower oil, epoxidized perilla oil, epoxidized lard oil, epoxidized tallow and epoxidized fish oils such as menhaden and sardine oil as well as epoxidized sperm oil. These compositions are readily available in that the naturally occurring ethylenically unsaturated materials can be epoxidized by methods well known in the art to provide compositions having varying amounts of oxirane substitution.

Other aliphatic alcohol esters of oxirane-substituted higher fatty acids such as mono- and dihydric alcohol esters wherein the alcohol portion of the ester is a mono- or dihydric aliphatic alcohol having 1-8 carbons or a dihydric aliphatic alcohol having 2-6 carbons are also contemplated. Suitable monohydric alcohols providing the alcohol moiety of the epoxy fatty acid esters include methyl, ethyl, propyl, isopropyl, butyl, isobutyl, amyl, isooamyl, hexyl, heptyl and octyl alcohols. Dihydric alcohols which may be employed to provide the alcohol moiety of the epoxy fatty acid ester include ethylene glycol, 1,2-propane diol, 1,3-propane diol, dimethyl ethylene glycol, trimethylene glycol, tetramethylene glycol, up to and including hexamethylene glycol. Polyhydric alcohol esters of the oxirane-containing fatty acids which can be employed to provide the oxirane-containing reactant include the epoxy higher fatty acid esters of tri-, tetra-, penta- and hexa-hydric alcohol esters of the fatty acid moiety. Included within this group are those aliphatic alcohols having 3-6 carbons and 3 or more alcohol groups. These alcohols include glycerol, erythritol, penta-erythritol and hexitols such as mannitol and sorbitol. Synthetic triglycerides such as epoxidized triolein, epoxidized trilinolein and epoxidized trilinolenin are also contemplated. Generally, esters of acids of the type such as epoxidized oleic acid, epoxidized linoleic acid and epoxidized linolenic acid are preferred.

Esters of epoxidized higher fatty alcohols with lower mono- and polycarboxylic aliphatic acids are also contemplated. Included in this group are 9,10-epoxy stearoyl acetate, di-(9,10-epoxystearoyl)maleate and di-(9-, 10-, 12-, 13-diepoxy stearoyl)adipate.

The hydroxyl supplying reactant can be selected from the group consisting of ethers and esters of aliphatic monohydric alcohols. Examples of compositions of this type are the alkyl phenol polyoxyalkylene glycol adducts such

as nonyl phenyl ethylene oxide condensation products wherein 6-12 mols of ethylene oxide are combined with each mol of nonyl phenol. The alkyl group on the benzeneoid ring of such composition can contain 8-14 carbons and can be either a straight or branch chain. Lower alkyl and alkenyl ethers such as the 1-4 carbon ethers of polyoxyalkylene glycols are also contemplated.

The esters of the polyoxyalkylene glycols include the higher fatty acid esters containing 10-22 carbons in the fatty acid portion of the molecule. These acids are obtained from naturally occurring fats and oils. Tall oil fatty acid esters of polyoxyethylene glycol having 12-18 oxyethylene groups are typical of the higher fatty acid esters of polyoxyalkylene compounds.

Typical structures of the adjacent hydroxyl and ether groups on the hydrocarbon chain which before reaction were occupied by the epoxy groups are as follows:

(A)



(B)



(C)



where X is H or aliphatic hydrocarbon radical of 8-14 carbons, n is 1-100, R<sub>1</sub> is an aliphatic hydrocarbon radical of 9-21 carbons, and R<sub>2</sub> is an aliphatic hydrocarbon radical of 1-6 carbons.

Generally, the compositions of the present invention will contain about 1-5 of the above groups.

While the compositions illustrated have for convenience been shown containing oxyethylene groups it should be understood that compositions made up of oxypropylene and oxybutylene groups are also encompassed by the invention.

As previously stated, the catalytic agent utilized in producing the compositions used in the present invention may be selected from the group consisting of strong Lewis acids, tertiary amines and alkali metal alcoholates. Suitable catalysts include Friedel-Crafts type catalysts such as the halides of boron, iron, aluminum, silicon, antimony, tin, arsenic, zinc, and zirconium. Also, tertiary amines such as benzyl dimethyl amine, lower C<sub>1</sub> through C<sub>4</sub> trialkyl amines and trialkyloamines are satisfactory catalysts as are potassium ethylate, sodium methylate, etc. Boron trifluoride and boron trifluoride complexes are preferred, although lower alkoxides of metals such as aluminum and titanium isopropoxides and isobutoxides are also satisfactory. A catalytic amount of about 0.5-7% based upon the epoxide depending upon the activity of the specific catalyst will ordinarily be employed.

The ratio of the oxirane-containing material to the alcohol composition which are combined is usually maintained so that there are sufficient hydroxyl groups to react with each epoxide group and insure that the degree of functionality in the reaction product is held at a minimum. If an excess of either reactant is to be employed, it is preferred that the hydroxy compound be present in an excess.

In order to prepare the lubricants suitable for use in the present invention, the above-described compositions are formed into a uniform aqueous dispersion by mild agitation. From about 0.5 to about 50%, and preferably from about 1.0 to about 10% by weight of the composition is combined with water.

The following examples illustrate the production and use of the above specified compositions in the present invention. These examples are presented merely for purposes of illustrating the present invention.

*Example I*

Epoxidized soybean oil having an oxirane content of 6.95% was added to 640 grams of ethoxylated nonyl phenol. The ethoxylated nonyl phenol is the condensation product of 9.5 mols of ethylene oxide condensed with one mol of nonyl phenol. Two hundred fifty grams of epoxidized oil was added to a dispersion of 8 grams of a boron trifluoride-ethyl Cellosolve complex in the ethoxylated nonyl phenol. The mixture was stirred and an exothermic reaction took place as the polyoxyethylene ether reacted with epoxidized oil. A milky white dispersion was then produced by mixing 20 grams of the material thus formed with 180 grams of water. This dispersion was evaluated for lubricity at a metal-metal interface in a "Baroid" oil well drilling mud tester in which a rotating metal ring is brought into contact with the surface of a metal block beneath the surface of the test solution. Pressure is applied to the block and is measured by means of a torque wrench. Seizure is indicated by monitoring an ammeter which measures the current drawn by the motor and noting the torque value at which it increases precipitately. Failure occurred at a value of 132 foot pounds as opposed to 53 foot pounds for a 10% solution of a diethanolammonium oleate-lauryl diethanol amide blend commonly used as an aqueous drawing compound.

*Example II*

A composition was formed by reacting 310 grams of ethoxylated nonylphenol (1.5 mols ethylene oxide) with 230 grams of epoxidized soybean oil in the presence of 1.25 grams of boron trifluoride etherate under reaction conditions such as those taught in Example I. The material formed by this reaction was not self-dispersible in water and was somewhat darker than that of Example I. However, dispersibility was restored by the addition of 10% of the reaction product of Example I and the material thus formed exhibited lubricating properties comparable to those obtained in Example I.

*Example III*

Four hundred ten grams of ethoxylated octyl phenol (43% by weight ethylene oxide) were reacted with 180 grams of epoxidized linseed oil (oxirane oxygen 9.03%) in the presence of 3 grams of tin tetrachloride. The procedure used was the same as that of Example I. This material exhibited properties almost identical to the properties of the material obtained in Example I, but was of a slightly darker color.

*Example IV*

Five hundred grams of ethoxylated oleyl alcohol (54% by weight ethylene oxide) were reacted with 385 grams of epoxidized sperm oil (oxirane oxygen 4.14%) in the presence of 4 grams of antimony pentachloride by a procedure as that taught in Example I. The resultant product was quite dark in color but exhibited desirable properties as a lubricant.

*Example V*

Seven grams of epoxidized soybean oil were reacted with 34 grams of ethoxylated dinonylphenol (73% by weight ethylene oxide) in the presence of 12 drops of boron trifluoride-Cellosolve complex by a procedure similar to that of Example I. The resultant material was a pasty liquid which showed desirable lubricating properties and also showed utility as a fluid-loss inhibitor in drilling muds indicating that it could be used in the lubrication of drilling bits in oil wells.

*Example VI*

Nine hundred sixty grams of epoxidized 2-ethylhexylsuccinate (oxirane oxygen 4.2%) were reacted with 610 grams of ethoxylated dodecyl mercaptan in the presence of 5 grams of boron trichloride by the procedure of

**Example I.** The product resulting from this reaction exhibited utility as a lubricant for drilling and cutting operations in ferrous metals.

Obviously, many modifications and variations of the invention as hereinbefore set forth may be made without departing from the spirit and scope thereof and, therefore, only such limitations should be imposed as are indicated in the appended claims.

I claim:

1. A method for improving the working properties of metals comprising: applying to a metal-metal interface an aqueous dispersion of an ester of a higher fatty acid, the fatty acyl chain of said ester having substituted on adjacent carbons hydroxyl groups and ether radicals, said ether radicals being selected from the group consisting of oxyalkylene ethers and oxyalkylene esters.
  2. The method of claim 1 wherein the aqueous dispersion contains from about 0.5% to about 50% of said ester.
  3. The process of claim 1 wherein the polyoxy alkylene compound contains about 40-90% by weight oxyalkylene groups.
  4. The process of claim 1 wherein the ester has a molecular weight of above about 200 and contains from about 1 to about 5 pairs of hydroxy groups and ether radicals.

5. The process of claim 1 wherein the ester is derived from a naturally occurring triglyceride.
  6. The process of claim 1, wherein the ester employed contains from about 1 to about 5 of the following groups



where Y is an alkylene group of 2-4 carbons, m is 1-100 and Z is selected from the group consisting of acyl, phenyl, phenyl alkyl, and lower alkyl groups.

7. The process of claim 1, wherein said ether radicals are ethers of alkoxylated alkyl phenols.

UNITED STATES PATENTS

### References Cited

|           |         |                   |       |             |
|-----------|---------|-------------------|-------|-------------|
| 3,242,200 | 3/1966  | Johnson           | ----- | 260-398     |
| 1,795,491 | 3/1931  | Johnson           | ----- | 252-49.5 X  |
| 3,024,198 | 3/1962  | Harrington et al. | 252   | -49.5 X     |
| 3,066,159 | 11/1962 | Groote            | ----- | 260-410.7 X |
| 3,117,929 | 1/1964  | McCoy et al.      | ----- | 252-49.5 X  |
| 3,202,607 | 8/1965  | Kock              | ----- | 252-49.5    |

DANIEL E. WYMAN, *Primary Examiner.*

W. H. CANNON, *Assistant Examiner*